

## UNITED STATES PATENT OFFICE

2,155,347

## ALLOY STEELS

Marcus A. Grossmann, Chicago, Ill., assignor to  
United States Steel Corporation, New York,  
N. Y., a corporation of New Jersey

No Drawing. Application October 22, 1936,  
Serial No. 107,104

2 Claims. (Cl. 75—126)

The present invention relates to alloy steels.

In the strict sense, steel may be said to be an alloy of iron and carbon. However, in a metallurgical sense, in which the term is used in this specification, an alloy steel is steel (that is, iron and carbon) alloyed with another chemical element or other chemical elements.

An object of the present invention is to produce an alloy steel which is well adapted to resist failure by fatigue, especially for use in highly stressed parts, such as springs.

A further object is to produce an alloy steel for general purposes which involves no special equipment in its manufacture and which has improved characteristics over steel as heretofore known and used.

A further object is to provide a steel well adapted for use in cushioning springs, which steel will effectually resist deterioration in service.

A further object is to provide an alloy steel in which the characteristics of titanium are utilized to advantage in the manufacture of alloy steels.

A further object is to provide an improved steel well adapted to meet the needs of commercial operation.

Further objects will appear as the description proceeds.

The present invention contemplates the accomplishment of the objects above referred to by providing a shallow hardening alloy steel. To the skilled steel manufacturer the term "shallow hardening alloy steel" has a definite significance, meaning a steel which, when heated to above its critical temperature and then cooled, has a relatively pronounced tendency to change rapidly from the austenitic to the pearlitic type of internal structure. Steel of fine grain structure tends to be shallow hardening, though of course certain alloy steels, even though they be fine grained, may not be shallow hardening in comparison with the steels for which invention is claimed herein. Of course it is possible to produce shallow hardening steel by using a very restricted amount of carbon, and such steel has its uses in the arts. The present invention is limited to steels in which the carbon content is equal to or greater than .45% by weight.

In defining the degree of shallow hardening contemplated in the present invention it may be observed that certain alloy steels, as for example nickel chromium steel, have characteristics differing from steels contemplated in the

present invention. As is well known, alloy steels as ordinarily known to metallurgists will, when heated to a temperature of say 1600 deg. F., form austenite, which is understood by metallurgists to be a solution of carbon in iron. As the steel is cooled from the temperature referred to, the structure changes, and when the steel reaches the neighborhood of about 900 deg. F. there is a tendency to form pearlite, which is a tough substance of low hardness. In the case of most alloy steels as now known and used, as for example the nickel chromium steel above referred to, the length of time in the temperature zone in the neighborhood of 900 deg. F. required for the formation of pearlite is in the neighborhood of 20 seconds. The temperature zone referred to may range from 1050 to 850 deg. F. In the case of the alloy steels forming the subject matter of the present invention, the period of time required in the 900 deg. zone referred to is in the neighborhood of 8 seconds. Considering a body of steel which has been heated to say about 1600 deg. F. and quenched in water, it will be readily understood that in the case of nickel chromium steel or the like the period of dwell in the 900 deg. zone referred to may be too short to form pearlite, but said period of dwell may be ample for the formation of pearlite in the composition of shallow hardening steels. In other words, using the example above referred to, the period of time in which the center of the member under test is in the temperature zone of 900 deg. F. above referred to may be less than 20 seconds but more than 8 seconds. In the event that pearlite has not formed in the quenching operation, the alloy steel, upon further cooling, will form martensite, which is a hard material. In the event that pearlite has formed in the center of the member under test in the quenching operation, this pearlite will retain its identity when the member under test has cooled to atmospheric temperature. The above example illustrates a measure which may be applied to define the degree of hardenability contemplated in the present invention. For convenience, the measure of hardenability may be expressed in connection with an alloy steel bar. The present invention contemplates a composition of alloy steel such that when a cylindrical bar of 1½ inches or more in diameter of homogeneous composition is heated to a temperature of approximately 1600 deg. F. and then quenched in still water at room temperature, the material at the axis of said bar will, upon cooling to room temperature, have a

Rockwell hardness of not more than 50-C. Ex-  
pressed in another way, and referring to the  
quenching of the alloy steel in oil, the present  
invention contemplates a composition alloy  
5 steel such that when a cylindrical bar of 1  
inch or more in diameter of homogeneous com-  
position is heated to a temperature of approxi-  
mately 1600 deg. F. and then quenched in still  
10 oil at room temperature, the material at the axis  
of said bar will have a Rockwell hardness of  
not more than 50-C.

It will be understood, of course, that the ref-  
erences immediately above made to bars of spec-  
ified diameters are merely for convenience of  
15 definition of one property of these steels. The  
steels, of course, are useful in members of all  
dimensions including small sections in which  
the steels harden through to their axes or mid-  
sections.

20 Titanium has the advantage that it produces  
fine grain structure and is relatively low in price.  
As is well known, the cheapest form of titanium  
on the market at the present time is that which  
has been reduced by treatment with carbon re-  
25 sulting in what is known as a high carbon ferro  
titanium. In some arts, the high carbon content  
is objectionable but in the manufacture of alloy  
spring steel in which the carbon content is rel-  
atively high, the high carbon content of the low-  
30 priced high carbon ferro titanium is not objec-  
tionable.

Titanium has the advantage that it tends to  
produce fine grain structure and shallow hard-  
35 ening over a relatively wide temperature range  
in the hardening operation. Moreover, when  
using titanium in the manufacture of alloy  
spring steel the amount of aluminum may be  
materially reduced from present practice in the  
melting operation to secure fine grain structure  
40 and shallow hardening.

45 In carrying out the present invention it is  
contemplated to use in the manufacture of the  
improved alloy steel a predominating amount of  
titanium either with or without other shallow  
hardening elements, such for example as vanadi-  
um or equivalent. Correspondingly, the present  
50 invention contemplates a relatively low amount  
of the deep hardening elements (such for exam-  
ple as manganese, chromium and/or nickel). The  
relative terms referred to in the preceding  
sentence have reference to the functions of the  
alloying elements referred to as commonly used  
55 in alloy steels in common use today.

Proceeding to a more specific definition of al-  
loying elements contemplated in the present in-  
55 vention, the following observations may be  
made:

60 Since titanium reaches its full effectiveness  
for grain refinement at approximately 0.06% by  
weight, a predominating amount of titanium in  
the alloy steel according to the present invention  
would be approximately 0.02 to 0.06% by weight.

65 Since vanadium reaches its full effectiveness  
at about 0.15% to 0.20%, a predominating  
amount of vanadium would be about 0.075 to  
0.20% by weight.

70 On the other hand, chromium may be said to  
have its greatest effectiveness at about 1.5% by  
weight, so that a predominating amount of  
chromium would be about .75%-1.5%.

75 Since manganese reaches its maximum effec-  
tiveness at about 2% by weight, a predominating  
amount of manganese would be about 1.25%-2%  
by weight.

Since nickel reaches its full effectiveness at  
about 3% to 4%, a predominating amount of  
nickel would be about 1%-4% by weight.

Therefore, expressing the purpose of the pres-  
ent invention in other language, it may be said 5  
that the present invention contemplates the use  
of titanium in the amount of 0.02 to 0.06% by  
weight, said element being used without chromi-  
um or manganese if preferred; or, if chromium  
be used, then with less than .75% by weight of 10  
chromium; or, if manganese be used, then with  
less than 1.25% of manganese. Expressed in  
still other language, certain advantages of the  
present invention will be had if the shallow 15  
hardening elements (for example titanium, with  
or without vanadium or equivalent) are used to a  
percentage equal to at least 50% of their fully  
effective amount in opposing hardening in  
quenched steels; and certain advantages of the  
present invention will be had if the deep harden- 20  
ing elements (for example chromium, manga-  
nese and/or nickel) are restricted to not more  
than 50% of their fully effective amounts as  
hardening agents in quenched steels. Another  
way of defining the limits of the materials con- 25  
templated in the present invention is by refer-  
ence to the "critical cooling rate" of the mate-  
rials. Critical cooling rate of steels may be de-  
fined as that rate above which a steel will harden  
in the cooling process and below which a steel 30  
will not harden. When the term "harden" is  
used in this connection it is intended to convey  
the meaning that the material of the steel be-  
comes the hard material "martensite". The  
present invention contemplates steels which 35  
when quenched in a quenching medium at at-  
mospheric temperature will just harden if it  
passes 1325 deg. F. at a rate above 50 deg. per  
second but below 150 deg. per second.

Those skilled in the art will understand that 40  
manganese is usually present in the manufac-  
ture of steel to the extent of about .2%-.5% by  
weight, since manganese is commonly used as a  
de-oxidizer in steel making; and for the same  
45 reason silicon is usually present in amounts of  
.2%.

Proceeding now to a still more specific recita-  
tion of analysis of steel falling within the scope  
of the present invention, the following example  
may be recited:

|                | Per cent   |
|----------------|------------|
| Carbon from    | .85 to .95 |
| Manganese from | .20 to .50 |
| Silicon from   | .10 to .35 |
| Chromium from  | .20 to .50 |
| Titanium from  | .03 to .06 |

Balance largely iron with traces of impurities.

It will be understood, of course, that the anal-  
ysis just noted is illustrative only, and the ob-  
jects of the present invention may be realized by  
proper balancing of shallow hardening elements  
against deep hardening elements. For example,  
the carbon may vary from .30% to 1%; the man-  
ganese may vary from .40% to 1.25%; the chro-  
mium may vary from 0 to .75%; the titanium  
may vary from 0.01% to 0.10%. A choice of  
the elements referred to, to provide a shallow  
hardening steel meeting the tests recited in this  
invention, will fall within the scope of this  
70 invention.

Anyone familiar with the manufacture of alloy  
steels has readily available to him information  
as to the constituents and the amounts thereof  
which must be used in producing the steels hav-  
ing the foregoing analyses.

- In arriving at the object of making a shallow hardening alloy steel, the present invention contemplates a steel of fine grain size. In referring to fine grain size it is to be understood that reference is had to the grain size of austenite, which is the structure composing the steel when the steel has been heated to a high temperature (for example 1600 deg. F.) preparatory to hardening by quenching. The term "fine grain" or "fine grain size" as used in this specification means from #5 to #8 on the ASTM chart of grain sizes. This may be further explained as meaning more than 12 grains per square inch when examined at a magnification of 100 diameters.
- 15 The fact is well known that fine grain size tends to shallow hardening. It is also well known that very fine grains, particularly #7 and #8, according to the ASTM chart, exhibit structural features known as abnormality, meaning thereby a particular distribution of the iron carbide (that is, cementite) observed in the carburizing test (McQuaid-Ehn carburizing test), which test is sometimes used in determining grain size.
- 20 In order to arrive at fine grain size (including abnormality) it has been common to add, in the furnace, in the ladle or in the molds, about one pound of aluminum per ton of steel. It has been discovered that if titanium be used as one of the shallow hardening elements, the amount of aluminum may be materially reduced. Titanium tends to produce fine grain structure and shallow hardening in steel over a relatively wide temperature range in the hardening operation.
- 25 As is well known, silicon is used in the manufacture of alloy quality steels for the purpose of combining with the oxygen and thereby removing said oxygen. An excess of silicon always ap-

pears in the finished steel of this type and may properly be considered to be a trace of impurity. Accordingly, in the appended claims the term "traces of impurities" will include this excess silicon.

The alloy steels forming the subject matter of this invention are characterized by a high degree of ductility, toughness, resiliency and resistance to shock and fatigue.

Though certain preferred analyses and steps have been recited in the foregoing specification, many modifications will occur to those skilled in the art. It is intended to cover all such modifications that fall within the scope of the appended claims.

What is claimed is:—

1. A shallow hardening alloy steel which is composed of the following ingredients substantially in the amounts specified:

|                | Per cent   | 20 |
|----------------|------------|----|
| Carbon from    | .85 to .95 |    |
| Manganese from | .20 to .50 |    |
| Chromium from  | .20 to .50 |    |
| Titanium from  | .03 to .06 | 25 |

Balance iron with traces of impurities.

2. An alloy steel characterized by a high degree of resilience and resistance to shock and fatigue which is composed of the following ingredients within the ranges specified and balanced against each other to produce a shallow hardening steel:

|                | Per cent     |    |
|----------------|--------------|----|
| Carbon from    | .45 to 1     |    |
| Manganese from | .40 to 1.25  |    |
| Chromium       | trace to .75 | 35 |
| Titanium from  | .01 to .10   |    |

Remainder iron with traces of impurities.

MARCUS A. GROSSMANN.